

July 10, 1928.

1,676,949

J. J. HIGGINS

METHOD OF SOLDERING LEADING-IN WIRES TO LAMP BASES

Filed April 21, 1923

FIG.1.

FIG.2.

FIG.3.



FIG.4.

FIG.5.

FIG.6.

FIG.7.



FIG.8.

FIG.9.

FIG.10.



INVENTOR

JOHN J. HIGGINS

BY

*J. J. Higgins*

ATTORNEY

## UNITED STATES PATENT OFFICE.

JOHN JOSEPH HIGGINS, OF EAST ORANGE, NEW JERSEY, ASSIGNOR TO WESTINGHOUSE LAMP COMPANY, A CORPORATION OF PENNSYLVANIA.

## METHOD OF SOLDERING LEADING-IN WIRES TO LAMP BASES.

Application filed April 21, 1923. Serial No. 633,798.

This invention relates to the manufacture of incandescent electric lamps and more particularly to the method of securing leading-in wires to the bases of such lamps.

5 An object of the invention is to provide a simple and practical method of securing a leading-in wire to a metallic base.

Another object is to provide a method in which a sequence of operations for securing 10 a leading-in wire to a base, may be readily adapted for automatic performance.

A further object of the invention is to provide a method for maintaining a quantity of fusible material in position, prior 15 to the fusing operation.

A further object of the invention is to provide a method for controlling the amount of fusible material employed to secure a leading-in wire to a base.

20 A still further object of the invention consists in the formation of a cavity in a body for the reception of a fusible material whereby a leading-in wire and said material may be properly juxtaposed for a fusing operation to secure the wire to the body.

The manufacture of incandescent electric lamps requires certain soldering operations, the leading-in wires or conductors of the lamp being usually connected with external 30 contacts for the purpose of permitting a flow of electrical current when the lamp is screwed, or otherwise inserted, into a socket of a lighting circuit. Lamps, as generally constructed, have one of the leading-in wires 35 thereof secured to a contact member which is insulated from the shell or metallic base. The insulated contact member is generally positioned at the lower end of the base and disposed axially thereof.

40 The other leading-in wire is usually soldered or otherwise secured to the external cylindrical surface of a threadless portion of the base of the lamp; that is, the connection that is made on the periphery of the 45 base, to distinguish from the axially disposed connection, may be termed a peripheral contact.

The present invention provides a method for facilitating the operation of securing the 50 peripheral disposed leading-in wire. Heretofore, the peripheral or circumferentially disposed leading-in wire of a lamp was soldered to the shell or base by suitably positioning the wire adjacent to the circumfer-

ence of the base and depositing an amount 55 of molten material thereon, a suitable flux being employed.

The above operation was a manual one and, although, when skillfully performed, resulted in satisfactory unions, the operations required did not lend themselves well 60 to automatic actuation.

Although the soldering of a leading-in wire to a base by manual operation appears 65 to be a simple one, the conditions attending upon the automatic soldering operations were such that great difficulty was experienced in obtaining a method which would be adaptable for mechanical performance.

70 Attempts have been made to automatically solder leading-in wires to the circumference of a base, and one difficulty which presented itself resided in the inability of the machine to deposit the proper amount of fusible material when making the connection. It will be appreciated that either too little or an excessive amount of material upon the wire would tend toward a defective union or present 75 an appearance which would be inconsistent with the manufacturing standard in the production of electric incandescent lamps. Furthermore, the deposit of an excessive amount of solder prevents the proper adjustment of the base within a socket.

80 It was also found difficult to properly position the wire prior to the soldering operation in order to maintain it in proper position for the soldering operation.

85 The present invention avoids the difficulties set forth above by providing an aperture in the base of a lamp and in temporarily securing a leading-in wire within the aperture by the insertion of a section of the solder to be subsequently used as the material 90 for securing the leading-in wire to the base. This solder is applied by first inserting the end of a rod of solder into the aperture and in severing a small section from the rod, the section being of such length as to slightly 95 project above the aperture. A soldering iron 100 may then be moved to make contact with the solder to fuse it and effect the connection of the leading-in wire to the base.

105 Another advantage is derived from the fact that, in the present method, the base is so positioned that, when the solder is in the molten state, it will, by reason of gravity,

flow along the leading-in wire and thus will more securely connect the wire to the shell or base of the lamp.

The method will be more readily understood when considered in connection with the accompanying drawings, in which

Figs. 1 to 10, inclusive, are side elevational views of a lamp base and a portion of a bulb at the various stages of operation of my 10 method of equipping the base with a leading-in wire.

A lamp to which the present method may be applied may comprise the usual bulb 11 having a screw base 12 cemented thereto. 15 Leading-in wire 13 may then be bent to form a loop 14, and a suitable drill 15 be operated to form an aperture 16. The aperture 16 may, if desired, be formed in a base prior to its application to the bulb. It may be desirable to press an aperture or cavity in the shell instead of drilling therethrough, or a plurality of properly disposed prongs may be stamped out of the shell and bent upwardly to receive a predetermined amount of 20 solder. The preferable method is, however, to drill through the base to produce the aperture 16, whereupon, the loop 14 may be inserted into the aperture as shown in Fig. 3. When the loop is thus positioned, the 25 end of a rod of solder 17 having a suitable flux applied thereto may be inserted into the aperture.

The rod of solder may then be severed to leave a small portion or section 18 disposed 30 within the aperture and in contact with the leading-in wire (see Fig. 7). The solder thus disposed may be readily fused by the application of a heated iron 19 which may be moved to make contact with the solder to 35 heat the same, and fuse it, with the result that a connection or deposit 21 is effected. By reason of the vertical position of the longitudinal axis of the lamp, the solder will flow downwardly and embed the greater 40 portion of leading-in wire adjacent to the outside of the base.

Although the present invention may be considered as having the operations thus performed semi-automatically, it will be understood that suitable mechanism may be provided for progressively operating upon the lamp to seal the wire thereto.

The looped portion of the leading-in wire may then be inserted into the hole, and the 55 end of the rod of solder may also be inserted and forced in contact with the leading-in wire, thus securely anchoring the leading-in wire in position. When the end of the solder has been properly disposed in 60 the aperture, it may be severed at a point adjacent to the base, so as to leave a small portion of the solder rod projecting from the aperture.

If desirable, instead of inserting the leading-in wire into the hole 16, the solder may

be inserted therein and the leading-in wire twisted around the projecting portion of the section 18 of solder, as shown in Fig. 10. Finally the soldering iron 19 may be operated to fuse the solder 18 to consolidate 7 the wire with the base.

It will be appreciated that, by reason of the present invention, the handling of the lamp for the automatic or semi-automatic soldering operation may be accomplished in 7 a simple and practical manner. Furthermore, by reason of the operation for severing the section 18 of solder from the rod, a predetermined amount of such material may be provided and a uniform union main- 8 tained.

Although the present description states one method of practicing my invention and the drawing illustrates an embodiment thereof, it is obvious that modifications may 8 be made therein without departing from the spirit and scope of the appended claims.

What is claimed is:

1. The method of soldering leading-in wire to a base which comprises bending a 9 leading-in wire to form a loop, drilling a hole in said base, positioning said loop in said hole, inserting an end of a rod of fusible material into said hole and in contact with said loop, severing said rod to permit a short section thereof to project from said hole, moving a heated member to fuse said section and positioning the lamp so as to permit a flow of the fused material along a portion of the length of said leading-in 10 wire.

2. The method of securing a leading-in wire to a base which comprises forming an aperture in said base, inserting said leading-in wire therein, positioning the base with its longitudinal axis vertical, applying a fusible material to a portion of the leading-in wire disposed in said aperture, fusing said material and permitting the fused material to flow along a portion of the leading-in wire adjacent to the aperture.

3. The method of soldering a leading-in wire to a base which comprises forming an aperture in a base, looping the end of a leading-in wire, inserting said loop in said 11 aperture, positioning the end of a rod of solder in said aperture, severing said rod to leave a portion of said solder projecting from said aperture and fusing said portion to secure said leading-in wire to the base. 12

4. The method of soldering a leading-in wire to a base which comprises forming an aperture in said base, disposing the end of a rod of fusible material in said aperture, severing said rod to leave a section thereof 12 projecting from said aperture, disposing a leading-in wire adjacent to said section and heating said material to secure said leading-in wire to the base.

5. The method of soldering a leading-in 13

wire to a base which comprises bending the end of a leading-in wire to loop form, drilling a hole in said base, inserting the end of a rod of fusible material into said hole, positioning said looped end of the wire adjacent said fusible material, severing said material to leave a relatively short portion thereof in said hole, applying a flux and heating said fusible material to secure the leading-in wire to the base.

5 6. The method of soldering a leading-in wire to a base which comprises drilling a hole in said base, inserting an end of a rod of fusible material into said hole, disposing the end of a leading-in wire adjacent to said fusible material, applying a flux and fusing said material to secure said leading-in wire to the base.

10 7. The method of soldering a leading-in wire to a base which comprises drilling a hole in said base, positioning the end of a leading-in wire within said hole, forcing the

end of a rod of solder into said hole and in contact with said leading-in wire, severing said rod to permit a short section thereof 25 to remain in said hole, applying a flux and moving a heated member to fuse said solder to secure the leading-in wire to said base.

8. The method of soldering a leading-in wire to a base which comprises drilling a hole through the wall of said base, looping the end of a leading-in wire, positioning said loop within said hole, inserting the end of a rod of solder into said hole and in contact with said leading-in wire, severing 30 said rod to permit a small section thereof to remain in said hole, applying a flux and fusing said positioned section to secure said leading-in wire to said base.

15 In testimony whereof, I have hereunto 40 subscribed my name this 20th day of April, 1923.

JOHN JOSEPH HIGGINS.